# EUROPEAN PATENT SPECIFICATION

(11) **EP 2 743 338 B1**
(45) Date of publication and mention of the grant of the patent: **29.03.2017**
(21) Application number: 12196743.4
(22) Date of filing: 12.12.2012
(51) Int. Cl.: C11D 3/20, C11D 11/00, C11D 17/00, C11D 17/04

(54) **Improved structuring with short non-polymeric, crystalline, hydroxyl-containing structuring agents**
Verbesserte Strukturierung mit kurzen nicht polymeren, kristallinen, hydroxylhaltigen Strukturmitteln
Structuration améliorée avec des agents structurants cristallins non polymères courts contenant de l'hydroxyle

(43) Date of publication of application: 18.06.2014
(73) Proprietor: The Procter & Gamble Company, Cincinnati, OH 45202 (US)
(72) Inventor: De Meirleir, Niels, 1932 St-Stevens-Woluwe (BE); Broeckx, Walter August Maria, 9290 Berlare (BE); Pellens, Linda, 3071 Erps-Kwerps (BE)
(74) Representative: Siddiquee, Sanaul Kabir

(56) References cited:
- EP-A1- 1 396 535
- EP-A1- 2 495 300
- EP-A1- 2 698 195
- WO-A1-2010/034736
- WO-A1-2011/031940

## Description

### FIELD OF THE INVENTION

Structuring premixes, comprising small particles of non-polymeric, crystalline, hydroxyl-containing structuring agent, have been found to be highly effective for structuring high surfactant liquid detergent compositions, and liquid detergent compositions comprising hydrophobic ingredients.

### BACKGROUND OF THE INVENTION

Aqueous structurant premixes comprising a non-polymeric, crystalline, hydroxyl-containing structuring agent, such as hydrogenated castor oil, are used to structure and thicken liquid compositions. While the non-polymeric, crystalline, hydroxyl-containing structuring agent can be melted and directly dispersed into a liquid composition, the structuring agent is usually first formed into a premix in order to both improve processibility, and to improve structuring efficacy. Hence, the molten structuring agent is generally first emulsified in water, and then crystallised to form an aqueous structuring premix. The resultant aqueous structuring premix is then used to structure liquid compositions, and also to increase the viscosity of such liquid compositions (see for example, WO2011031940).

In recent years, liquid compositions, for use around the household, have undergone "compaction", whereby the concentration of actives such as surfactants and cleaning polymers has increased while the recommended dosage has correspondingly decreased. Such compact liquid compositions, since they are richer in actives, are costly to make. Liquid compositions are usually structured, in order to provide a richer, more luxurious consumer experience. However, structuring ingredients also add to the cost of the liquid composition. Hence, there is a need to increase the efficacy of structurants, such that lower levels need to be added in order to arrive at the desired level of structuring.

### SUMMARY OF THE INVENTION

The present invention relates to a liquid composition, comprising an aqueous structuring premix, wherein said aqueous structuring premix comprises water and particles, said particles comprising non-polymeric, crystalline, hydroxyl-containing structuring agent, wherein at least 80% by number of the particles have a length less than 6 microns; wherein the liquid composition is a liquid detergent composition, comprising at least one surfactant, present at a level of from 1 to 70% by weight of the liquid composition; and wherein the liquid composition comprises from 0.01wt% to 2wt% of the non-polymeric, crystalline, hydroxyl-containing structuring agent, introduced via the aqueous structuring premix.

The present invention further relates to a unit dose article, comprising such liquid detergent compositions, wherein the liquid detergent composition comprises less than 20 % by weight of water, and is encapsulated in a water-soluble film.

### DETAILED DESCRIPTION OF THE INVENTION

Aqueous structuring premixes, comprising a non-polymeric, crystalline, hydroxyl-containing structuring agent, typically structured by forming a physical network in the liquid composition. Such aqueous structuring premixes had previously been formed by emulsifying the structuring agent at a temperature at or above the melt point of the structuring agent, and then slowly reducing the temperature to crystallise and grow strands of the structuring agent. Hence, the physical network, which provides the structuring benefit, was previously present in the aqueous structuring premix.

It has been surprisingly discovered, that when an emulsion of the non-polymeric, crystalline, hydroxyl-containing structuring agent is rapidly cooled, the aqueous structuring premix comprises predominately small particles of the non-polymeric, crystalline, hydroxyl-containing structuring agent. Moreover, it has been surprisingly discovered that such small particles of non-polymeric, crystalline, hydroxyl-containing structuring agent are highly effective for structuring liquid detergent compositions comprising higher levels of surfactant.

Since the aqueous structuring premix of use in the present invention is more efficient at structuring such liquid detergent compositions, less structuring premix needs to be added to deliver the desired level of structuring. Therefore, less water is introduced by the structuring premix, into the liquid composition. As such, the structuring premix of use in the present invention is particularly suitable for low water liquid detergent compositions, such as those intended to be encapsulated in water-soluble films to form unit dose articles.

As defined herein, "essentially free of" a component means that the component is present at a level of less that 15%, preferably less 10%, more preferably less than 5%, even more preferably less than 2% by weight of the respective premix or composition. Most preferably, "essentially free of" a component means that no amount of that component is present in the respective premix, or composition.

As defined herein, "stable" means that no visible phase separation is observed for a premix kept at 25°C for a period of at least two weeks, preferably at least four weeks, more preferably at least a month or even more preferably greater than four months, as measured using the Floc Formation Test, described in USPA 2008/0263780 A1.

All percentages, ratios and proportions used herein are by weight percent of the respective premix or composition, unless otherwise specified. All average values are calculated "by weight" of the respective premix, composition, or components thereof, unless otherwise expressly indicated.

Unless otherwise noted, all component, premix, or composition levels are in reference to the active portion of that component, premix, or composition, and are exclusive of impurities, for example, residual solvents or by-products, which may be present in commercially available sources of such components or compositions.

All measurements are performed at 25°C unless otherwise specified.

### The aqueous structuring premix:

The aqueous structuring premix of use in the present invention comprises water, which forms the balance of the structuring premix, after the weight percentage of all of the other ingredients are taken into account. Water is preferably present at a level of from 45% to 97%, more preferably from 55% to 93%, even more preferably from 65% to 87% by weight of the aqueous structuring premix.

The non-polymeric crystalline, hydroxyl functional structuring agent is emulsified into the water. Non-polymeric crystalline, hydroxyl functional structuring agents comprise a crystallisable glyceride. Preferably, the non-polymeric, crystalline, hydroxyl-containing structuring agent comprises, or even consists of, hydrogenated castor oil (commonly abbreviated to "HCO") or derivatives thereof.

The aqueous structuring premix of use in the present invention comprises a non-polymeric, crystalline, hydroxyl-containing structuring agent in the form of particles. The particles are typically rod-like or thread-like. The non-polymeric, crystalline, hydroxyl-containing structuring agent is preferably present at a level of from 2% to 10%, more preferably from 3% to 8%, even more preferably from 4% to 6% by weight of the aqueous structuring premix.

At least 80% by number of the particles, comprising non-polymeric, crystalline, hydroxyl-containing structuring agent, have a length of less than 6 microns. Preferably, at least 80% by number of the particles have a length of from 0.25 to 6 microns. The particle length is defined as the maximum axial length of the particle. It has been found that such small particles result in improved structuring, when added to liquid detergent compositions comprising high levels of surfactant. Preferably at least 90%, preferably 95% by number of the particles have a length less than 6 microns. Preferably, at least 90%, preferably 95% by number of the particles have a length greater than 0.25 microns, and less than 6 microns. Preferably at least 70%, preferably 80%, more preferably 90% by number of the particles have a length less than 2 microns. Preferably at least 70%, preferably 80%, more preferably 90% by number of the particles have a length greater than 0.25 microns, and less than 2 microns. Surprisingly, the short particles, having a length less than 2 microns have been found to be particularly effective for structuring compact liquid detergent compositions.

As mentioned earlier, the non-polymeric, crystalline, hydroxyl-containing structuring agent is preferably hydrogenated castor oil. Castor oil is a triglyceride vegetable oil, comprising predominately ricinoleic acid, but also oleic acid and linoleic acids. When hydrogenated, it becomes castor wax, otherwise known as hydrogenated castor oil. The hydrogenated castor oil may comprise at least 85% by weight of the castor oil of ricinoleic acid. Preferably, the hydrogenated castor oil comprises glyceryl tris-12-hydroxystearate (CAS 139-44-6). In a preferred embodiment, the hydrogenated castor oil comprises at least 85%, more preferably at least 95% by weight of the hydrogenated castor oil of glyceryl tris-12-hydroxystearate. However, the hydrogenated castor oil composition can also comprise other saturated, or unsaturated linear or branched esters. In a preferred embodiment, the hydrogenated castor oil has a melting point in the range of from 45°C to 95 °C, as measured using ASTM D3418 or ISO 11357. The hydrogenated castor oil may have a low residual unsaturation and will generally not be ethoxylated, as ethoxylation tends to reduce the melting point temperature to an undesirable extent. By low residual unsaturation, we herein mean an iodine value of 20 of less, preferably 10 or less, more preferably 3 or less. Those skilled in the art would know how to measure the iodine value using commonly known techniques.

The aqueous structuring premix of use in the present invention preferably comprises a surfactant, added as an emulsifying agent in order to improve emulsification of the non-polymeric, crystalline, hydroxyl-containing structuring agent, and to stabilize the resultant droplets. When added, the surfactant is preferably added at a concentration above the critical micelle concentration (c.m.c) of the surfactant. When the non-polymeric, crystalline, hydroxyl-containing structuring agent is emulsified into an aqueous phase containing these micelles, a portion of the non-polymeric, crystalline, hydroxyl-containing structuring agent is transferred to the micelles, to form droplets that are stabilised by the micelles. The surfactant may be present in the aqueous structuring premix at a level of from 1% to 45%, preferably from 4% to 37%, more preferably from 9% to 29% of the aqueous structuring premix. The weight percentage of surfactant is measured, based on the weight percentage of the surfactant anion. That is, excluding the counterion. When using more than 25% by weight of the structuring premix of an anionic surfactant, it is preferred to thin the surfactant using an organic solvent, in addition to water.

Detersive surfactants are preferred, i.e. a surfactant that provides detersive effect on hard surfaces or fabrics. For example, a detersive surfactant may provide greasy stain or soil/clay stain removal from treated surfaces or substrates. For instance, the detersive surfactant may provide fabric cleaning benefits during a washing cycle. The surfactant can be selected from the group comprising anionic, non-ionic, cationic and zwitterionic surfactants. Although any suitable surfactant can be used, an anionic surfactant is preferred. Preferably, the anionic surfactant is selected from the group consisting of: alkyl sulphonate, alkylbenzene sulphonate, alkyl sulphate, alkyl alkoxylated sulphate and mixtures thereof. Depending on the pH, either the acid form or salt form of the anionic surfactant can be used. However, while the acid form of the anionic surfactant can be used, the anionic surfactant is preferably neutralized, before the addition of the non-polymeric, crystalline, hydroxyl-containing structuring agent.

Preferred sulphonate detersive surfactants include alkyl benzene sulphonate, preferably C₁₀₋₁₃ alkyl benzene sulphonate. Suitable alkyl benzene sulphonate (LAS) is preferably obtained by sulphonating commercially available linear alkyl benzene (LAB); suitable LAB includes low 2-phenyl LAB, such as those supplied by Sasol under the tradename Isochem® or those supplied by Petresa under the tradename Petrelab®, other suitable LAB include high 2-phenyl LAB, such as those supplied by Sasol under the tradename Hyblene®. A preferred anionic detersive surfactant is alkyl benzene sulphonate that is obtained by DETAL catalyzed process, although other synthesis routes, such as HF, may also be suitable.

Preferred sulphate detersive surfactants include alkyl sulphate, preferably C₈₋₁₈ alkyl sulphate, or predominantly C₁₂ alkyl sulphate.

Another preferred sulphate detersive surfactant is alkyl alkoxylated sulphate, preferably alkyl ethoxylated sulphate, preferably a C₈₋₁₈ alkyl alkoxylated sulphate, preferably a C₈₋₁₈ alkyl ethoxylated sulphate, preferably the alkyl alkoxylated sulphate has an average degree of alkoxylation of from 0.5 to 20, preferably from 0.5 to 10, preferably the alkyl alkoxylated sulphate is a C₈₋₁₈ alkyl ethoxylated sulphate having an average degree of ethoxylation of from 0.5 to 10, preferably from 0.5 to 7, more preferably from 0.5 to 5 and most preferably from 0.5 to 3.

The alkyl sulphate, alkyl alkoxylated sulphate and alkyl benzene sulphonates may be linear or branched, substituted or un-substituted.

The aqueous structuring premix may contain additional surfactant in addition to anionic surfactants. In particular, the aqueous structuring premix may comprise additional surfactant selected from: nonionic surfactant; cationic surfactant; amphoteric surfactant; zwitterionic surfactant; and mixtures thereof.

The aqueous structuring premix may further comprise a pH adjusting agent. Any known pH-adjusting agents can be used, including alkalinity sources as well as acidifying agents of either inorganic type and organic type, depending on the desired pH.

The pH-adjusting agent is typically present at concentrations from 0.2% to 20%, preferably from 0.25% to 10%, more preferably from 0.3% to 5.0% by weight of the aqueous structuring premix.

Inorganic alkalinity sources include but are not limited to, water-soluble alkali metal hydroxides, oxides, carbonates, bicarbonates, borates, silicates, metasilicates, and mixtures thereof; water-soluble alkali earth metal hydroxides, oxides, carbonates, bicarbonates, borates, silicates, metasilicates, and mixtures thereof; water-soluble boron group metal hydroxides, oxides, carbonates, bicarbonates, borates, silicates, metasilicates, and mixtures thereof; and mixtures thereof. Preferred inorganic alkalinity sources are sodium hydroxide, and potassium hydroxide and mixtures thereof, most preferably inorganic alkalinity source is sodium hydroxide. Although not preferred for ecological reasons, water-soluble phosphate salts may be utilized as alkalinity sources, including pyrophosphates, orthophosphates, polyphosphates, phosphonates, and mixtures thereof.

Organic alkalinity sources include but are not limited to, primary, secondary, tertiary amines, and mixtures thereof. Other organic alkalinity sources are alkanolamine or mixture of alkanolamines. Suitable alkanolamines may be selected from the lower alkanol mono-, di-, and trialkanolamines, such as monoethanolamine; diethanolamine or triethanolamine. Higher alkanolamines have higher molecular weight and may be less mass efficient for the present purposes. Mono- and dialkanolamines are preferred for mass efficiency reasons. Monoethanolamine is particularly preferred, however an additional alkanolamine, such as triethanolamine, can be useful in certain embodiments as a buffer. Most preferred alkanolamine used herein is monoethanol amine.

Inorganic acidifying agents include but are not limited to, HF, HCl, HBr, HI, boric acid, phosphoric acid, phosphonic acid, sulphuric acid, sulphonic acid, and mixtures thereof. Preferred inorganic acidifying agent is boric acid.

Organic acidifying agents include but are not limited to, substituted and substituted, branched, linear and/or cyclic C₁ to C₃₀ carboxyl acids, and mixtures thereof.

The aqueous structuring premix may optionally comprise a pH buffer. In some embodiments, the pH is maintained within the pH range of from 5 to 11, or from 6 to 9.5, or from 7 to 9. Without wishing to be bound by theory, it is believed that the buffer stabilizes the pH of the aqueous structuring premix, thereby limiting any potential hydrolysis of the HCO structurant. However, buffer-free embodiments can be contemplated and when HCO hydrolyses, some 12-hydroxystearate may be formed, which is also capable of structuring, though to a lesser extent than HCO. In certain preferred buffer-containing embodiments, the pH buffer does not introduce monovalent inorganic cations, such as sodium, into the structuring premix. The preferred buffer is the monethanolamine salt of boric acid. However embodiments are also contemplated in which the buffer is is free from any deliberately added sodium, boron or phosphorus. In some embodiments, MEA neutralized boric acid may be present at a level of from 0% to 5%, from 0.5% to 3%, or from 0.75% to 1% by weight of the aqueous structuring premix.

As already noted, alkanolamines such as triethanolamine and/or other amines can be used as buffers, provided that alkanolamine is first added in an amount sufficient for the primary structurant emulsifying purpose of neutralizing the acid form of anionic surfactants, or the anionic surfactant has previously been neutralized by another means.

The aqueous structuring premix may further comprise a non-aminofunctional organic solvent. Non-aminofunctional organic solvents are organic solvents which contain no amino functional groups. Preferred non-aminofunctional organic solvents include monohydric alcohols, dihydric alcohols, polyhydric alcohols, glycerol, glycols including polyalkylene glycols such as polyethylene glycol, and mixtures thereof. More preferred non-aminofunctional organic solvents include monohydric alcohols, dihydric alcohols, polyhydric alcohols, glycerol, and mixtures thereof. Highly preferred are mixtures of non-aminofunctional organic solvents, especially mixtures of two or more of the following: lower aliphatic alcohols such as ethanol, propanol, butanol, isopropanol; diols such as 1,2-propanediol or 1,3-propanediol; and glycerol. Also preferred are mixtures of propanediol and diethylene glycol. Such mixtures preferably contain no methanol or ethanol.

Preferable non-aminofunctional organic solvents are liquid at ambient temperature and pressure (i.e. 21°C and 1 atmosphere), and comprise carbon, hydrogen and oxygen. Non-aminofunctional organic solvents may be present when preparing the structurant premix, or added directly to the liquid composition.

The aqueous structuring premix may also comprise a preservative or biocide, especially when it is intended to store the premix before use.

### Liquid compositions comprising the aqueous structuring premix:

The aqueous structuring premix, of use in the present invention, is useful for structuring liquid compositions. Hence, a liquid composition can comprise the aqueous structuring premix. The liquid compositions of the present invention typically comprise from 0.01wt% to 2wt%, preferably from 0.03wt% to 1wt%, more preferably from 0.05wt% to 0.5wt% of the non-polymeric, crystalline, hydroxyl-containing structuring agent, introduced via the aqueous structuring premix.

Suitable liquid compositions include: products for treating fabrics, including laundry detergent compositions and rinse additives; hard surface cleaners including dishwashing compositions, floor cleaners, and toilet bowl cleaners. The aqueous structuring premix of use in the present invention is particularly suited for liquid detergent compositions. Such liquid detergent compositions comprise sufficient detersive surfactant, so as to provide a noticeable cleaning benefit. Most preferred are liquid laundry detergent compositions, which are capable of cleaning a fabric, such as in a domestic washing machine.

As used herein, "liquid composition" refers to any composition comprising a liquid capable of wetting and treating a substrate, such as fabric or hard surface. Liquid compositions are more readily dispersible, and can more uniformly coat the surface to be treated, without the need to first dissolve the composition, as is the case with solid compositions. Liquid compositions can flow at 25°C, and include compositions that have an almost water like viscosity, but also include "gel" compositions that flow slowly and hold their shape for several seconds or even minutes.

A suitable liquid composition can include solids or gases in suitably subdivided form, but the overall composition excludes product forms which are non-liquid overall, such as tablets or granules. The liquid compositions preferably have densities in the range from of 0.9 to 1.3 grams per cubic centimetre, more preferably from 1.00 to 1.10 grams per cubic centimetre, excluding any solid additives but including any bubbles, if present.

Preferably, the liquid composition comprises from 1% to 95 % by weight of water, non-aminofunctional organic solvent, and mixtures thereof. For compact liquid compositions, the composition preferably comprises from 15% to 70%, more preferably from 20% to 50%, most preferably from 25% to 45% by weight of water, non-aminofunctional organic solvent, and mixtures thereof. Alternatively, the liquid composition may be a low water liquid composition. Such low water liquid compositions can comprise less than 20%, preferably less than 15%, more preferably less than 10 % by weight of water.

The liquid composition of the present invention may comprise from 2% to 40 %, more preferably from 5 % to 25 % by weight of a non-aminofunctional organic solvent.

The liquid composition can also be encapsulated in a water soluble film, to form a unit dose article. Such unit dose articles comprise a liquid composition of the present invention, wherein the liquid composition is a low water liquid composition, and the liquid composition is enclosed in a water-soluble or dispersible film.

The unit dose article may comprise one compartment, formed by the water-soluble film which fully encloses at least one inner volume, the inner volume comprising the low water liquid composition. The unit dose article may optionally comprise additional compartments comprising further low water liquid compositions, or solid compositions. A multi-compartment unit dose form may be desirable for such reasons as: separating chemically incompatible ingredients; or where it is desirable for a portion of the ingredients to be released into the wash earlier or later. The unit-dose articles can be formed using any means known in the art.

Unit dose articles, wherein the low water liquid composition is a liquid laundry detergent composition are particularly preferred.

Suitable water soluble pouch materials include polymers, copolymers or derivatives thereof. Preferred polymers, copolymers or derivatives thereof are selected from the group consisting of: polyvinyl alcohols, polyvinyl pyrrolidone, polyalkylene oxides, acrylamide, acrylic acid, cellulose, cellulose ethers, cellulose esters, cellulose amides, polyvinyl acetates, polycarboxylic acids and salts, polyaminoacids or peptides, polyamides, polyacrylamide, copolymers of maleic/acrylic acids, polysaccharides including starch and gelatin, natural gums such as xanthum and carragum. More preferred polymers are selected from polyacrylates and water-soluble acrylate copolymers, methylcellulose, carboxymethylcellulose sodium, dextrin, ethylcellulose, hydroxyethyl cellulose, hydroxypropyl methylcellulose, maltodextrin, polymethacrylates, and most preferably selected from polyvinyl alcohols, polyvinyl alcohol copolymers and hydroxypropyl methyl cellulose (HPMC), and combinations thereof.

As mentioned earlier, the liquid composition of the present invention can be a liquid detergent composition, preferably a liquid laundry detergent composition. Liquid detergent compositions comprise a surfactant, to provide a detergency benefit. The liquid detergent compositions of the present invention may comprise from 1% to 70%, preferably from 5% to 60%, more preferably from 10% to 50%, most preferably from 15% to 45% by weight of a detersive surfactant. Suitable detersive surfactants can be selected from the group consisting of: anionic, nonionic surfactants and mixtures thereof. The preferred weight ratio of anionic to nonionic surfactant is from 100:0 (i.e. no nonionic surfactant) to 5:95, more preferably from 99:1 to 1:4, most preferably from 5:1 to 1.5:1.

The liquid detergent compositions of the present invention preferably comprise from 1 to 50%, more preferably from 5 to 40%, most preferably from 10 to 30% by weight of one or more anionic surfactants. Preferred anionic surfactant are selected from the group consisting of: C11-C18 alkyl benzene sulphonates, C10-C20 branched-chain and random alkyl sulphates, C10-C18 alkyl ethoxy sulphates, mid-chain branched alkyl sulphates, mid-chain branched alkyl alkoxy sulphates, C10-C18 alkyl alkoxy carboxylates comprising 1-5 ethoxy units, modified alkylbenzene sulphonate, C12-C20 methyl ester sulphonate, C10-C18 alpha-olefin sulphonate, C6-C20 sulphosuccinates, and mixtures thereof. However, by nature, every anionic surfactant known in the art of detergent compositions may be used, such as those disclosed in "Surfactant Science Series", Vol. 7, edited by W. M. Linfield, Marcel Dekker. The detergent compositions preferably comprise at least one sulphonic acid surfactant, such as a linear alkyl benzene sulphonic acid, or the water-soluble salt form of the acid.

The detergent compositions of the present invention preferably comprise up to 30%, more preferably from 1 to 15%, most preferably from 2 to 10% by weight of one or more nonionic surfactants. Suitable nonionic surfactants include, but are not limited to C12-C18 alkyl ethoxylates ("AE") including the so-called narrow peaked alkyl ethoxylates, C6-C12 alkyl phenol alkoxylates (especially ethoxylates and mixed ethoxy/propoxy), block alkylene oxide condensate of C6-C12 alkyl phenols, alkylene oxide condensates of C8-C22 alkanols and ethylene oxide/propylene oxide block polymers (Pluronic^{®}-BASF Corp.), as well as semi polar nonionics (e.g., amine oxides and phosphine oxides). An extensive disclosure of suitable nonionic surfactants can be found in U.S. Pat. 3,929,678.

The liquid detergent composition may also include detergent ingredients selected from the group consisting of: additional surfactants selected from amphoteric, zwitterionic, cationic surfactant, and mixtures thereof; enzymes; enzyme stabilizers; amphiphilic alkoxylated grease cleaning polymers; clay soil cleaning polymers; soil release polymers; soil suspending polymers; bleaching systems; brighteners; hueing dyes; particulates; perfume and other odour control agents, including perfume delivery systems; hydrotropes; suds suppressors; fabric care perfumes; pH adjusting agents; dye transfer inhibiting agents; preservatives; non-fabric substantive dyes; and mixtures thereof. The aqueous structuring premix is particularly suited for structuring liquid detergent compositions which comprise hydrophobic parts or groups, such as detergent ingredient selected from the group consisting of: amphiphilic alkoxylated grease cleaning polymers; clay soil cleaning polymers; soil release polymers; soil suspending polymers; optical brighteners; particulates; perfume and other odour control agents, including perfume delivery systems; suds suppressors; fabric care perfumes; and mixtures thereof. More preferably, the liquid detergent composition comprises a detergent ingredient selected from the group consisting of: amphiphilic alkoxylated grease cleaning polymers; brighteners and mixtures thereof.

Preferably, the liquid detergent composition comprises a brightener, such as a fluorescent brightener. Fluorescent brighteners absorb light from the UV-spectrum, and emit visible light. Particularly preferred, are fluorescent brighteners which emit light in the blue or violet spectrum, having a wavelength of from 380 to 450 nm.

Brighteners which are useful in the present invention can be classified into subgroups, which include, but are not necessarily limited to, derivatives of stilbene, pyrazoline, carboxylic acid, methinecyanines, dibenzothiophene-5,5-dioxide, azoles, 5- and 6-membered-ring heterocycles, and mixtures thereof. Examples of such brighteners are disclosed in "The Production and Application of Fluorescent Brightening Agents", M. Zahradnik, Published by John Wiley & Sons, New York (1982). Specific nonlimiting examples of optical brighteners which are useful in the present compositions are those identified in U.S. Pat. No. 4,790,856 and U.S. Pat. No. 3,646,015.

Suitable fluorescent brighteners include: C.I. fluorescent brightener 9, C.I. fluorescent brightener 49, C.I. fluorescent brightener 260, and mixtures thereof.

Fluorescent brightener 9 (2,2'-(1,2-Ethenediyl)bis[5-[[4,6-bis(phenylamino)-1,3,5-triazin-2-yl]amino] disodium salt, CAS 133-66-4) has the following structure:

C.I Fluorescent brightener 49 (disodium 2,2'-([1,1'-biphenyl]-4,4'-diyldivinylene)bis(benzenesulphonate);2,2'-([1,1'-Biphenyl]-4,4'-diyldi-2,1-ethenediyl)bis-benzenesulfonic acid disodium salt, CAS 27344-41-8) has the following structure:

C.I. fluorescent brightener 260 (2,2-(1,2-ethenediyl)bis[5-[[4-(4-morpholinyl)-6-(phenylamino)-1,3,5-triazin-2-yl]amino]-benzenesulfonic acid], disodium salt, CAS: 73071-63-3), preferably in alpha-crystalline form, has the following structure:

The brightener is typically added in micronized particulate form, having a weight average primary particle size of from 3 to 30 micrometers, from 3 micrometers to 20 micrometers, or from 3 to 10 micrometers, typically as part of a slurry.

The fluorescent brightener may be added at a level of from 0.01, from 0.05, or even from 0.1, up to a level of 0.5 or even 0.75 wt%.

The brightener may be loaded onto clay to form a particle.

Suitable amphiphilic alkoxylated grease cleaning polymers are any alkoxylated polymers having balanced hydrophilic and hydrophobic properties such that they remove grease particles from fabrics and surfaces. Specific embodiments of the amphiphilic alkoxylated grease cleaning polymers of the present invention comprise a core structure and a plurality of alkoxylate groups attached to that core structure.

The core structure may comprise a polyalkylenimine structure comprising, in condensed form, repeating units of formulae (I), (II), (III) and (IV): wherein # in each case denotes one-half of a bond between a nitrogen atom and the free binding position of a group A¹ of two adjacent repeating units of formulae (I), (II), (III) or (IV); * in each case denotes one-half of a bond to one of the alkoxylate groups; and A¹ is independently selected from linear or branched C₂-C₆-alkylene; wherein the polyalkylenimine structure consists of 1 repeating unit of formula (I), x repeating units of formula (II), y repeating units of formula (III) and y+1 repeating units of formula (IV), wherein x and y in each case have a value in the range of from 0 to 150; where the average weight average molecular weight, Mw, of the polyalkylenimine core structure is a value in the range of from 60 to 10,000 g/mol.

The core structure may alternatively comprise a polyalkanolamine structure of the condensation products of at least one compound selected from N-(hydroxyalkyl)amines of formulae (I.a) and/or (I.b), wherein A are independently selected from C₁-C₆-alkylene; R¹, R¹*, R², R²*, R³, R³*, R⁴, R⁴*, R⁵ and R⁵* are independently selected from hydrogen, alkyl, cycloalkyl or aryl, wherein the last three mentioned radicals may be optionally substituted; and R⁶ is selected from hydrogen, alkyl, cycloalkyl or aryl, wherein the last three mentioned radicals may be optionally substituted.

The plurality of alkylenoxy groups attached to the core structure are independently selected from alkylenoxy units of the formula (V) wherein * in each case denotes one-half of a bond to the nitrogen atom of the repeating unit of formula (I), (II) or (IV); A² is in each case independently selected from 1,2-propylene, 1,2-butylene and 1,2-isobutylene; A³ is 1,2-propylene; R is in each case independently selected from hydrogen and C₁-C₄-alkyl; m has an average value in the range of from 0 to 2; n has an average value in the range of from 20 to 50; and p has an average value in the range of from 10 to 50.

Specific embodiments of the amphiphilic alkoxylated grease cleaning polymers may be selected from alkoxylated polyalkylenimines having an inner polyethylene oxide block and an outer polypropylene oxide block, the degree of ethoxylation and the degree of propoxylation not going above or below specific limiting values. Specific embodiments of the alkoxylated polyalkylenimines according to the present invention have a minimum ratio of polyethylene blocks to polypropylene blocks (n/p) of 0.6 and a maximum of 1.5(x+2y+1)^{1/2}. Alkoxykated polyalkyenimines having an n/p ratio of from 0.8 to 1.2(x+2y+1)^{1/2} have been found to have especially beneficial properties.

The alkoxylated polyalkylenimines according to the present invention have a backbone which consists of primary, secondary and tertiary amine nitrogen atoms which are attached to one another by alkylene radicals A and are randomly arranged. Primary amino moieties which start or terminate the main chain and the side chains of the polyalkylenimine backbone and whose remaining hydrogen atoms are subsequently replaced by alkylenoxy units are referred to as repeating units of formulae (I) or (IV), respectively. Secondary amino moieties whose remaining hydrogen atom is subsequently replaced by alkylenoxy units are referred to as repeating units of formula (II). Tertiary amino moieties which branch the main chain and the side chains are referred to as repeating units of formula (III).

The polyalkylenimine backbone consisting of the nitrogen atoms and the groups A¹, preferably has an average molecular weight Mw of from 60 to 10,000 g/mole, more preferably from 100 to 8,000 g/mole and most preferably from 500 to 6,000 g/mole.

The sum (x+2y+1) corresponds to the total number of alkylenimine units present in one individual polyalkylenimine backbone and thus is directly related to the molecular weight of the polyalkylenimine backbone. The values given in the specification however relate to the number average of all polyalkylenimines present in the mixture. The sum (x+2y+2) corresponds to the total number amino groups present in one individual polyalkylenimine backbone.

The radicals A¹ connecting the amino nitrogen atoms may be identical or different, linear or branched C₂-C₆-alkylene radicals, such as 1,2-ethylene, 1,2-propylene, 1,2-butylene, 1,2-isobutylene,1,2-pentanediyl, 1,2-hexanediyl or hexamethylen. A preferred branched alkylene is 1,2-propylene. Preferred linear alkylene are ethylene and hexamethylene. A more preferred alkylene is 1,2-ethylene.

The hydrogen atoms of the primary and secondary amino groups of the polyalkylenimine backbone are replaced by alkylenoxy units of the formula (V).

In this formula, the variables preferably have one of the meanings given below:
A² in each case is selected from 1,2-propylene, 1,2-butylene and 1,2-isobutylene; preferably A² is 1,2-propylene. A³ is 1,2-propylene; R in each case is selected from hydrogen and C₁-C₄-alkyl, such as methyl, ethyl, n-propyl, isopropyl, n-butyl, isobutyl and tert.-butyl; preferably R is hydrogen. The index m in each case has a value of 0 to 2; preferably m is 0 or 1; more preferably m is 0. The index n has an average value in the range of from 20 to 50, preferably in the range of from 22 to 40, and more preferably in the range of from 24 to 30. The index p has an average value in the range of from 10 to 50, preferably in the range of from 11 to 40, and more preferably in the range of from 12 to 30.

Preferably the alkylenoxy unit of formula (V) is a non-random sequence of alkoxylate blocks. By non-random sequence it is meant that the [-A²-O-]ₘ is added first (i.e., closest to the bond to the nitrgen atom of the repeating unit of formula (I), (II), or (III)), the [-CH₂-CH₂-O-]ₙ is added second, and the [-A³-O-]ₚ is added third. This orientation provides the alkoxylated polyalkylenimine with an inner polyethylene oxide block and an outer polypropylene oxide block.

The substantial part of these alkylenoxy units of formula (V) is formed by the ethylenoxy units - [CH₂-CH₂-O)]ₙ- and the propylenoxy units -[CH₂-CH₂(CH₃)-O]ₚ-. The alkylenoxy units may additionally also have a small proportion of propylenoxy or butylenoxy units -[A²-O]ₘ-, i.e. the polyalkylenimine backbone saturated with hydrogen atoms may be reacted initially with small amounts of up to 2 mol, especially from 0.5 to 1.5 mol, in particular from 0.8 to 1.2 mol, of propylene oxide or butylene oxide per mole of NH- moieties present, i.e. incipiently alkoxylated.

This initial modification of the polyalkylenimine backbone allows, if necessary, the viscosity of the reaction mixture in the alkoxylation to be lowered. However, the modification generally does not influence the performance properties of the alkoxylated polyalkylenimine and therefore does not constitute a preferred measure.

The amphiphilic alkoxylated grease cleaning polymers are present in the detergent and cleaning compositions of the present invention at levels ranging from 0.05% to 10% by weight of the composition. Embodiments of the compositions may comprise from 0.1% to 5% by weight. More specifically, the embodiments may comprise from 0.25 to 2.5% of the grease cleaning polymer.

### Process for making the structuring premix:

The aqueous structuring premix of use in the present invention can be made using a process comprising the steps of: making an emulsion comprising a non-polymeric, crystalline, hydroxyl-containing structuring agent in water, at a first temperature of from 80 °C to 98 °C; cooling the emulsion to a second temperature of from 10 °C to 60 °C, in a period of from 10 seconds to 10 minutes; maintaining the emulsion at the second temperature for at least 2 minutes.

The emulsion comprises droplets of non-polymeric, crystalline, hydroxyl-containing structuring agent, preferably hydrogenated castor oil (HCO), in molten form. The droplets preferably have a mean diameter of from 0.1 microns to 4 microns, more preferably from 1 micron to 3.5 microns, even more preferably from 2 microns to 3.5 microns, most preferably from 2.5 microns to 3 microns. The mean diameter is measured at the temperature at which emulsification is completed.

The emulsion can be prepared by providing a first liquid comprising, or even consisting of, the non-polymeric, crystalline, hydroxyl-containing structuring agent in molten form and a second liquid comprising water. The first liquid is emulsified into the second liquid. This is typically done by combining the first liquid and second liquid together and passing them through a mixing device.

The second liquid preferably comprises from 50% to 99%, more preferably from 60% to 95%, most preferably from 70% to 90% by weight of water. The second liquid may also comprise a surfactant, in order to improve emulsification. In a preferred embodiment, at least 1% by weight of the second liquid, preferably 1% to 50%, more preferably 5% to 40%, most preferably 10 to 30% by weight of the second liquid comprises a surfactant. The surfactant can be selected from the group comprising anionic, cationic, non-ionic, zwitterionic surfactants, or mixtures thereof. Preferably, the surfactant is an anionic surfactant, more preferably alkylbenzene sulphonate, most preferably linear alkylbenzene sulfonate. It should be understood that the surfactant is present in the second liquid at a concentration such that the emulsion produced is droplets of non-polymeric, crystalline, hydroxyl-containing structuring agent, present in a primarily water continuous phase, not a primarily surfactant continuous phase.

The surfactant can be added either in the acid form or as a neutralized salt. The second liquid can comprise a neutralizing agent, particularly when the surfactant is added in the acid form. By 'neutralizing agent', we herein mean a substance used to neutralize an acidic solution, such as formed when the surfactant is added in its acid form. Preferably, the neutralizing agent is selected from the group consisting of: sodium hydroxide, C₁-C₅ ethanolamines, and mixtures thereof. A preferred neutralizing agent is a C₁-C₅ ethanolamine, more preferably monoethanolamine.

The second liquid can comprise a preservative. Preferably the preservative is an antimicrobial. Any suitable preservative can be used, such as one selected from the 'Acticide' series of antimicrobials, commercially available from Thor Chemicals, Cheshire, UK.

The first liquid and the second liquid are combined to form an emulsion at the first temperature. The first temperature is from 80°C to 98°C, preferably from 85°C to 95°C, more preferably from 87.5°C to 92.5°C, to form the emulsion.

Preferably, the first liquid is at a temperature of 70°C of higher, more preferably between 70°C and 150°C most preferably between 75°C and 120°C, immediately before combining with the second liquid. This temperature range ensures that the non-polymeric, crystalline, hydroxyl-containing structuring agent is molten so that the emulsion is efficiently formed. However, a temperature that is too high results in discoloration or even degradation of the non-polymeric, crystalline, hydroxyl-containing structuring agent.

The second liquid is typically at a temperature of from 80°C to 98°C, preferably from 85°C to 95°C, more preferably from 87.5°C to 92.5°C, before being combined with the first liquid. That is, at or close to, the first temperature.

The ratio of non-polymeric, crystalline, hydroxyl-containing structuring agent to water in the emulsion can be from 1:50 to 1:5, preferably 1:33 to 1:7.5, more preferably 1:20 to 1:10. In other words the ratio of non-polymeric, crystalline, hydroxyl-containing structuring agent to water, as the two liquid streams are combined, for instance, upon entering a mixing device, can be from 1:50 to 1:5, preferably 1:33 to 1:7.5, more preferably 1:20 to 1:10.

The process to make the emulsion can be a continuous process or a batch process. By being continuous, down-time between runs is reduced, resulting in a more cost and time efficient process. By 'continuous process' we herein mean continuous flow of the material through the apparatus. By 'batch processes' we herein mean where the process goes through discrete and different steps. The flow of product through the apparatus is interrupted as different stages of the transformation are completed, i.e. discontinuous flow of material.

Without being bound by theory, it is believed that the use of a continuous process provides improved control of the emulsion droplet size, as compared to a batch process. As a result, a continuous process typically results in more efficient production of droplets having the desired mean size, and hence a narrower range of droplet sizes. Batch production of the emulsion generally results in larger variation of the droplet size produced, due to the inherent variation in the degree of mixing occurring within the batch tank. Variability can arise due to the use and placement of the mixing paddle within the batch tank. The result is zones of slower moving liquid (and hence less mixing and larger droplets), and zones of faster moving liquid (and hence more mixing and smaller droplets). Those skilled in the art will know how to select appropriate mixing devices to enable a continuous process. Furthermore, a continuous process will allow for faster transfer of the emulsion to the cooling step. The continuous process will also allow for less premature cooling, that can occur in a batch tank before transfer to the cooling step.

The emulsion can be prepared using any suitable mixing device. The mixing device typically uses mechanical energy to mix the liquids. Suitable mixing devices can include static and dynamic mixer devices. Examples of dynamic mixer devices are homogenizers, rotor-stators, and high shear mixers. The mixing device could be a plurality of mixing devices arranged in series or parallel in order to provide the necessary energy dissipation rate.

In one embodiment, the emulsion is prepared by passing the first and second liquids through a microchannel mixing device. Microchannel mixing devices are a class of static mixers. Suitable microchannel mixing devices can be selected from the group consisting of: split and recombine mixing devices, staggered herringbone mixers, and mixtures thereof. In a preferred embodiment, the micro-channel mixing device is a split and recombine mixing device.

Preferably, the emulsion is formed by combining the ingredients via high energy dispersion, having an energy dissipation rate of from 1 x 10² W/Kg to 1 x 10⁷ W/Kg, preferably from 1 x 10³ W/Kg to 5 x 10⁶ W/Kg, more preferably from 5 x 10⁴ W/Kg to 1 x 10⁶ W/Kg.

Without being bound by theory, it is believed that high energy dispersion reduces the emulsion size and increases the efficiency of the crystal growth in later steps.

In a second step the emulsion is cooled to a second temperature of from 10°C to 60°C, preferably from 15°C to 55°C, more preferably from 25°C to 50°C. Without wishing to be bound by theory, it is believed that this cooling step increases the crystallinity of the non-polymeric, crystalline, hydroxyl-containing structuring agent. The emulsion is preferably cooled as quickly as possible. For instance, the emulsion can be cooled to the second temperature in a period of from 10 s to 10 minutes, preferably in a period of less than 5 minutes, more preferably less than 2 minutes.

The emulsion can be cooled to the second temperature by any suitable means, such as by passing it through a heat exchanger device. Suitable heat exchanger devices can be selected from the group consisting of: plate and frame heat exchanger, shell and tube heat exchangers, and combinations thereof.

The emulsion can be passed through more than one heat exchanger device. In this case the second and subsequent heat exchanger devices are typically arranged in series with respect to the first heat exchanger. Such an arrangement of heat exchanger devices can be used to control the cooling profile of the emulsion.

The emulsion is maintained at a temperature of from 10 °C to 60 °C, preferably from 15°C to 55°C, more preferably from 25°C to 50°C, for a period of from 2 to 30 minutes, preferably from 5 to 20 minutes, more preferably from 10 to 15 minutes.

The process may comprise a further step of storing the aqueous structuring premix at a storage temperature of from 10°C to 30°C, preferably from 15°C to 24°C. In this temperature range, the aqueous structuring premix is sufficiently stable to be stored for extended periods before use.

The aqueous structuring premix formed from the process comprises little or no spherulites of the non-polymeric, crystalline, hydroxyl-containing structuring agent. It is believed that such spherulites are highly inefficient at structuring, and providing viscosity. Since the process produces little or no spherulites, it is believed that more non-polymeric, crystalline, hydroxyl-containing structuring agent is available for forming particles which are more effective at structuring than spherulites.

Any suitable means can be used for incorporating the aqueous structuring premix into a liquid composition, including static mixers, and through the use of over-head mixers, such as typically used in batch processes.

Preferably, the aqueous structuring premix is added after the incorporation of ingredients that require high shear mixing. More preferably, the aqueous structuring premix is the last ingredient incorporated into the liquid composition. The aqueous structuring premix is preferably incorporated into the liquid composition using low shear mixing. Preferably, the aqueous structuring premix is incorporated into the liquid composition using average shear rates of less than 1000s⁻¹, preferably less than 500s⁻¹, more preferably less than 200s⁻¹. The residence time of mixing is preferably less than 20s, more preferably less than 5s, more preferably less than Is. The shear rate and residence time is calculated according to the methods used for the mixing device, and is usually provided by the manufacturer. For instance, for a static mixer, the average shear rate is calculated using the equation: $\dot{γ} = \frac{{ν}_{pipe}}{{D}_{pipe}} ∗ {{ν}_{f}}^{- {/}_{2} 3}$ where:
*v_{f}* is the void fraction of the static mixer (provided by the supplier)
*Dₚᵢₚₑ* is the internal diameter of the pipe comprising the static mixer elements *vₚᵢₚₑ* is the average velocity of the fluid through a pipe having internal diameter *Dₚᵢₚₑ*, calculated from the equation: ${ν}_{pipe} = \frac{4 Q}{{{πD}_{pipe}}^{2}}$
*Q* is the volume flow rate of the fluid through the static mixer.

For a static mixer, the residence time is calculated using the equation: $residence time = \frac{{{πD}_{pipe}}^{2} {ν}_{f} L}{4 Q}$ where:
*L* is the length of the static mixer.

### METHODS:

### A) pH measurement:

The pH is measured on the neat composition, at 25°C, using a Santarius PT-10P pH meter with gel-filled probe (such as the Toledo probe, part number 52 000 100), calibrated according to the instructions manual.

### B) Rheology:

An AR-G2 rheometer from TA Instruments is used for rheological measurements, with a 40mm standard steel parallel plate, 300µm gap. All measurements, unless otherwise stated, are conducted according to the instruction manual, at steady state shear rate, at 25°C.

### C) Method of measuring the length of the particles of non-polymeric, crystalline, hydroxyl-containing structuring agent:

The aqueous structuring premix was analysed using Atomic force microscopy (AFM). The sample was prepared using the following procedure: The single side polished Si wafer (<100>, 381micron thickness, 2 nm native oxide, sourced from IDB Technologies, UK) is first cracked or cut into a piece of approximate dimensions 20 x 20 mm. The aqueous structuring premix is applied liberally to the Si wafer, using a cotton bud (Johnson & Johnson, UK). The paste-coated wafer is placed into a lidded poly(styrene) Petri dish (40 mm diameter, 10 mm height, Fisher Scientific, UK) and left for 5 minutes in air under ambient conditions (18°C, 40-50 % RH). The Petri dish is then filled with H₂O (HPLC grade, Sigma-Aldrich, UK) and the sample is left in the immersed conditions for approximately 1 hour. Following this, a cotton bud is used to remove the paste which has floated up away from the Si wafer surface, whilst the Si wafer was still immersed under HPLC grade H₂O. The Si wafer is then removed from the Petri dish and rinsed with HPLC grade H₂O. Subsequently, the Si wafer is dried in a fan oven at 35 °C for 10 min.

The wafer surface is then imaged as follows: The Si wafer is mounted in an AFM (NanoWizard II, JPK Instruments) and imaged in air under ambient conditions (18°C, 40-50 % RH) using a rectangular Si cantilever with pyramidal tip (PPP-NCL, Windsor Scientific, UK) in Intermittent Contact Mode. The image dimensions are 20 micron by 20 micron, the pixel density is set to 1024 x 1024, and the scan rate is set to 0.3 Hz, which corresponded to a tip velocity of 12 micron /s.

The resultant AFM image is analysed as follows: The AFM image is opened using ImageJ, version 1.46 (National Institute of Health, downloadable from: http://rsb.info.nih.gov/ij/). In the "Analyze" menu, the scale is set to the actual image size in microns, 20 µm by 20 µm. 20 particles, which do not contact the image edge, are selected at random. Using the "freehand line" function from the ImageJ Tools menu, the selected particles are each traced, and the length is measured (menu selections: "Plugins" / "Analyze" / "Measure and Set Label" / "Length"). In any size distribution calculations, particles of length less than 0.25 microns are not counted.

Three sets of measurements (sample preparation, AFM measurement and image analysis) are made, the results averaged.

### D) Energy Dissipation rate:

In a continuous process comprising a static emulsification device, the energy dissipation rate is calculated by measuring the pressure drop over the emulsification device, and multiplying this value by the flow rate, and then dividing by the active volume of the device. In the case where an emulsification is conducted via an external power source, such as a batch tank or high shear mixer, the energy dissipation is calculated via the following Formula 1 (Kowalski, A. J., 2009., Power consumption of in-line rotor-stator devices. Chem. Eng. Proc. 48, 581.); ${P}_{f} = {P}_{T} + {P}_{F} + {P}_{L}$

Wherein *P_{T}* is the power required to rotate the rotor against the liquid, *P_{F}* is the additional power requirements from the flow of liquid and *P_{L}* is the power lost, for example from bearings, vibration, noise etc.

### E) Rheology measurement:

Unless otherwise specified, the viscosity is measured using an Anton Paar MCR 302 rheometer (Anton Paar, Graz, Austria), with a cone and plate geometry having an angle of 2°, and a gap of 206 microns. The shear rate is held constant at a shear rate of 0.01s⁻¹, until steady state is achieved, then the viscosity is measured. The shear rate is then measured at 0.0224s⁻¹, 0.05s⁻¹, 0.11s⁻¹, 0.25s⁻¹, 0.55s⁻¹, 0.255s⁻¹, 2.8s⁻¹, 6.25s⁻¹, 14s⁻¹, 31.2s⁻¹, 70s⁻¹, waiting 10 seconds at each shear rate before each measurement is taken. All measurements were done on 20 °C.

### EXAMPLES:

Aqueous structuring premix A, of use in the present invention, was prepared in a continuous process, using the following procedure:
Hydrogenated castor oil was melted to form a first liquid at 90 +/- 5 °C. A second liquid, comprising 16.7 wt% linear alkylbenzene sulphonic acid (HLAS) and 3.34 wt% monoethanolamine, in water, was prepared at 90 +/- 5 °C. The first liquid was emulsified into the second liquid at a ratio of 4:96, via a continuous process, by combining the liquids and passing through a split-and-recombine static mixer, consisting of 11 steps and an inner diameter of 0.6mm (Ehrfeld, Wendelsheim, Germany) at a flow rate of 10 Kg/hr, to form an emulsion at 86°C. The resultant average emulsion size was 2.88 microns.

1 Kg/hr of the fluid was diverted to a heat exchanger, which comprised 3m of coiled 1/8" stainless steel tubing, followed by 2m of coiled 1/4" stainless steel tubing suspending in a water bath, which was used to cool the emulsion to a temperature of 45°C in less than 2 minutes. The fluid was then passed through a residence time unit, which comprised 6m of coiled 1/8" stainless steel tubing, followed by 4.6m of coiled 3/8" stainless steel tubing suspending in a water bath, which was used to maintain the fluid at a temperature of 45°C for 18 minutes, in order to form the particles of non-polymeric, crystalline, hydroxyl-containing structuring agent.

Comparative aqueous structuring premix B was prepared in a batch process, using the following procedure:
A liquid, comprising 6.7 wt% linear alkylbenzene sulphonic acid (HLAS) and 3.34 wt% monoethanolamine, in water, was prepared at 90 +/- 5 °C. Particulated hydrogenated castor oil was slowly dispersed into the liquid at a ratio of 4:96, in a batch process under agitation. Once molten, the hydrogenated castor oil is emulsified into the liquid. The emulsion was then slowly cooled at a rate 1°C/min, until a temperature of 40°C was reached. The aqueous structuring premix was then transferred to a storage tank and allowed to cool to room temperature.

The resultant aqueous structuring premixes: premix A of use in the invention, and comparative premix B, both had the following composition:

| | wt% |
|---|---|
| Monoethanolamine | 3.2 |
| Linear alkylbenzene sulphonic acid (HLAS) | 16.0 |
| Hydrogenated castor oil (HCO) | 4.0 |
| Water | 76.8 |

However, because of the different making processes, premix A, of use in the invention, comprised a greater proportion of small particles of the non-polymeric, crystalline, hydroxyl-containing structuring agent:

| Particle length (microns) | Aqueous premix A | Aqueous premix B (comparative) |
|---|---|---|
| | % particles | % particles |
| <2 | 100 | 57.50 |
| 2 - 4 | 0 | 7.50 |
| 4 - 6 | 0 | 7.50 |
| 6 - 8 | 0 | 10.00 |
| 8 - 10 | 0 | 5.00 |
| 10 - 12 | 0 | 5.00 |
| 12 - 14 | 0 | 0.00 |
| 14 - 16 | 0 | 0.00 |
| 16 - 18 | 0 | 2.50 |
| 18 - 20 | 0 | 0.00 |
| >20 | 0 | 5.00 |

Liquid compositions, having the following composition, and comprising either aqueous structuring premix A of use in the invention, or comparative aqueous structuring premix B, were prepared:

| Ingredient | Liquid composition A | Liquid composition B (Comparative) |
|---|---|---|
| | wt% | wt% |
| Linear Alkylbenzene sulphonic acid¹ | 8.2 | 8.2 |
| C12-14 alkyl ethoxy 3 sulphate Na salt | 2.8 | 2.8 |
| C12-14 alkyl 7-ethoxylate | 0.4 | 0.4 |
| C14-15 alkyl 7-ethoxylate | 4.9 | 4.9 |
| C12-18 Fatty acid | 3.5 | 3.5 |
| Sodium Cumene sulphonate | 1.0 | 1.0 |
| Citric acid | 3.4 | 3.4 |
| Ethoxysulfated Hexamethylene Diamine Dimethyl Quat | 1.0 | 1.0 |
| Soil Suspending Alkoxylated Polyalkylenimine Polymer² | 0.4 | 0.4 |
| PEG-PVAc Polymer³ | 0.5 | 0.5 |
| Di Ethylene Triamine Penta (Methylene Phosphonic acid, Na salt) | 0.3 | 0.3 |
| Fluorescent brightener 9 | 0.1 | 0.1 |
| 1,2 Propanediol | 1.3 | 1.3 |
| Ethanol | 1.2 | 1.2 |
| Aqueous structuring premix A (of use in the invention) | 10 | - |
| Aqueous structuring premix B (comparative) | - | 10 |
| Perfume | 0.9 | 0.9 |
| Sodium Hydroxide | 4.0 | 4.0 |
| Monoethanolamine | 0.4 | 0.4 |
| Protease enzyme (Purafect Prime®, 40.6 mg active/g)⁴ | 0.6 | 0.6 |
| Amylase enzyme (Termamyl Ultra®, 25.4mg active/g)⁵ | 0.05 | 0.05 |
| Amylase enzyme (Natalase®, 29.26mg active/g)⁵ | 0.1 | 0.1 |
| Mannanase enzyme (Mannaway®, 11mg active/g)⁵ | 0.06 | 0.06 |
| Xyloglucanase enzyme (Whitezyme®, 20mg active/g)⁵ | 0.06 | 0.06 |
| Water and minors (antifoam, aesthetics,...) | To 100 parts | |

| | | |
|---|---|---|
| ¹ Weight percentage of Linear Alkylbenzene sulfonic acid includes that which added to the composition via the premix ² 600 g/mol molecular weight polyethylenimine core with 20 ethoxylate groups per -NH. ³ PEG-PVA graft copolymer is a polyvinyl acetate grafted polyethylene oxide copolymer ⁴ Product of Genencor International, Palo Alto, California, USA ⁵ Products of Novozymes, Bagsvaerd, Denmark | | |

The resultant shear viscosities (measured at 0.2 s⁻¹), for treatment composition A, comprising the aqueous structuring premix of use in the present invention, and treatment composition B, comprising the comparative aqueous structuring premix, are given below:

| | shear viscosity (at 0.2 s⁻¹) |
|---|---|
| Liquid composition A, comprising premix A (of the invention) | 7.7 |
| Liquid composition B, comprising premix B (comparative) | 4.6 |

The following are non-limiting examples of aqueous structuring premixes of use in the present invention, which can be made using the process described herein:

| Ingredient | Aqueous structuring premix C | Aqueous structuring premix D | Aqueous structuring premix E | Aqueous structuring premix F | Aqueous structuring premix G |
|---|---|---|---|---|---|
| | wt% | wt% | wt% | wt% | wt% |
| Softened water | 73.55 | 75.1 | 73.6 | 74.6 | 75.6 |
| Monoethanolamine | 3.2 | 3.2 | 3.2 | 3.2 | 3.2 |
| Linear alkylbenzene sulphonic acid (HLAS) (<20% 2-phenyl isomers) | 16 | - | - | 16 | 16 |
| Linear alkylbenzene sulphonic acid (HLAS) (>20% 2-phenyl isomers) | - | 16 | 16 | - | - |
| Hydrogenated Castor Oil (HCO) | 6 | 4 | 5 | 4 | 4 |
| 1,2 propanediol | 1.05 | - | 2 | 2 | - |
| Urea | - | - | - | - | 1 |
| Acticide | 0.2 | 0.2 | 0.2 | 0.2 | 0.2 |

The aqueous structuring premixes, of use in the invention, can be added to unstructured treatment compositions, to form structured treatment compositions, as described below:

| Ingredient | Liquid composition C | Liquid composition D |
|---|---|---|
| | wt% | wt% |
| Linear Alkylbenzene sulphonic acid¹ | 7.5 | 10.5 |
| C12-14 alkyl ethoxy 3 sulphate Na salt | 2.6 | - |
| C12-14 alkyl ethoxy 3 sulphate MEA salt | - | 8.5 |
| C12-14 alkyl 7-ethoxylate | 0.4 | 7.6 |
| C14-15 alkyl 7-ethoxylate | 4.4 | - |
| C12-18 Fatty acid | 3.1 | 8 |
| Sodium Cumene sulphonate | 0.9 | - |
| Citric acid | 3.2 | 2.8 |
| Ethoxysulphated Hexamethylene Diamine Dimethyl Quat | 1 | 2.1 |
| Soil Suspending Alkoxylated Polyalkylenimine Polymer² | 0.4 | |
| PEG-PVAc Polymer³ | 0.5 | 0.8 |
| Di Ethylene Triamine Penta (Methylene Phosphonic acid, Na salt) | 0.3 | - |
| Hydroxyethane diphosphonic acid | - | 1.5 |
| Fluorescent Whitening Agent | 0.1 | 0.3 |
| 1,2 Propanediol | 3.9 | 7.5 |
| Diethylene Glycol | - | 3.5 |
| Sodium Formate | 0.4 | 0.4 |
| Hydrogenated castor oil (HCO)⁶ | 0.38 | 0.75 |
| Perfume | 0.9 | 1.7 |
| Sodium Hydroxide | To pH 8.4 | - |
| Monoethanolamine | 0.3 | To pH 8.1 |
| Protease enzyme | 0.4 | 0.7 |
| Amylase enzyme | - | 0.7 |
| Mannanase enzyme | 0.1 | 0.2 |
| Xyloglucanase enzyme | - | 0.1 |
| Pectate lyase | 0.1 | - |
| Water and minors (antifoam, aesthetics,...) | To 100 parts | |

| | | |
|---|---|---|
| ⁶ From an aqueous structuring premix of use in the invention | | |

Alternatively, the aqueous structuring premixes, of use in the invention, can be added to low water unstructured treatment compositions, to form structured low water treatment compositions, as described below:

| Ingredient | Liquid composition E | Liquid composition F | Liquid composition G |
|---|---|---|---|
| | wt% | wt% | wt% |
| Linear Alkylbenzene sulphonic acid¹ | 15 | 17 | 19 |
| C12-14 alkyl ethoxy 3 sulphonic acid | 7 | 8 | - |
| C12-15 alkyl ethoxy 2 sulphonic acid | - | - | 9 |
| C14-15 alkyl 7-ethoxylate | - | 14 | - |
| C12-14 alkyl 7-ethoxylate | 12 | - | - |
| C12-14 alkyl-9-ethoxylate | - | - | 15 |
| C12-18 Fatty acid | 15 | 17 | 5 |
| Citric acid | 0.7 | 0.5 | 0.8 |
| Polydimethylsilicone | - | 3 | - |
| Soil Suspending Alkoxylated Polyalkylenimine Polymer² | 4 | - | 7 |
| Hydroxyethane diphosphonic acid | 1.2 | - | - |
| Diethylenetriamine Pentaacetic acid | - | - | 0.6 |
| Ethylenediaminediscuccinic acid | - | - | 0.6 |
| Fluorescent Whitening Agent | 0.2 | 0.4 | 0.2 |
| 1,2 Propanediol | 16 | 12 | 14 |
| Glycerol | 6 | 8 | 5 |
| Diethyleneglycol | - | - | 2 |
| Hydrogenated castor oil (HCO)⁶ | 0.15 | 0.25 | 0.1 |
| Perfume | 2.0 | 1.5 | 1.7 |
| Perfume microcapsule | - | 0.5 | - |
| Monoethanolamine | Up to pH 8 | Up to pH 8 | Up to pH 8 |
| Protease enzyme | 0.05 | 0.075 | 0,12 |
| Amylase enzyme | 0.005 | - | 0.01 |
| Mannanase enzyme | 0.01 | - | 0.005 |
| xyloglucanase | - | - | 0.005 |
| Water and minors (antifoam, aesthetics, stabilizers etc.) | To 100 parts | To 100 parts | To 100 parts |

The resultant low water treatment compositions can be encapsulated in water-soluble film, to form water-soluble unit-dose articles.

## Claims

1. A liquid composition, comprising an aqueous structuring premix,
wherein said aqueous structuring premix comprises water and particles, said particles comprising non-polymeric, crystalline, hydroxyl-containing structuring agent, wherein at least 80% by number of the particles have a length less than 6 microns;
wherein the liquid composition is a liquid detergent composition, comprising at least one surfactant, present at a level of from 1 to 70% by weight of the liquid composition; and wherein the liquid composition comprises from 0.01wt% to 2wt% of the non-polymeric, crystalline, hydroxyl-containing structuring agent, introduced via the aqueous structuring premix.

2. The liquid composition according to claim 1, wherein the liquid detergent composition further comprises a detergent ingredients selected from the group consisting of: additional surfactants selected from amphoteric, zwitterionic, cationic surfactant, and mixtures thereof; enzymes; enzyme stabilizers; amphiphilic alkoxylated grease cleaning polymers; clay soil cleaning polymers; soil release polymers; soil suspending polymers; bleaching systems; optical brighteners; hueing dyes; particulates; perfume and other odour control agents, including perfume delivery systems; hydrotropes; suds suppressors; fabric care perfumes; pH adjusting agents; dye transfer inhibiting agents; preservatives; non-fabric substantive dyes; and mixtures thereof.

3. The liquid composition according to any preceding claims, wherein at least 90%, preferably 95% by number of the particles have a length less than 6 microns.

4. The liquid composition according to any preceding claims, wherein the non-polymeric, crystalline, hydroxyl-containing structuring agent is hydrogenated castor oil.

5. A unit dose article, comprising a liquid detergent composition according to any of claims 1 to 2, wherein the liquid detergent composition comprises less than 20 % by weight of water, and is encapsulated in a water-soluble film.

## Patentansprüche

1. Flüssige Zusammensetzung, umfassend eine wässrige strukturierende Vormischung,
wobei die wässrige strukturierende Vormischung Wasser und Teilchen umfasst, wobei die Teilchen nichtpolymeres, kristallines, hydroxylhaltiges Strukturierungsmittel umfassen, wobei mindestens 80 % der Teilchen, bezogen auf die Anzahl, eine Länge von weniger als 6 Mikrometern besitzen;
wobei die flüssige Zusammensetzung eine flüssige Waschmittelzusammensetzung ist, die mindestens ein Tensid umfasst, das in einer Konzentration von 1 bis 70 Gew.-% der flüssigen Zusammensetzung vorhanden ist; und
wobei die flüssige Zusammensetzung zu 0,01 Gew.-% bis 2 Gew.-% das nichtpolymere, kristalline, hydroxylhaltige Strukturierungsmittel umfasst, das durch die wässrige strukturierende Vormischung eingebracht wird.

2. Flüssige Zusammensetzung nach Anspruch 1, wobei die flüssige Waschmittelzusammensetzung ferner einen Waschmittelbestandteil umfasst, ausgewählt aus der Gruppe bestehend aus: zusätzlichen Tensiden, ausgewählt aus amphoterem, zwitterionischem, kationischem Tensid und Mischungen davon; Enzymen; Enzymstabilisatoren; amphiphilen alkoxylierten fettreinigenden Polymeren; Lehmschmutz entfernenden Polymeren; Schmutzabweisungspolymeren; Schmutzsuspendierpolymeren; Bleichmittelsystemen; optischen Aufhellern; Abtönungsfarbstoffen; Partikeln; Duftstoff- und anderen Geruchsunterdrückungsmitteln, einschließlich Duftstoffabgabesystemen; Hydrotropika; Schaumunterdrückern; Stoffpflegeduftstoffen; pH-Einstellmitteln; Farbstoffübertragungshemmern; Konservierungsmitteln; Nicht-Gewebesubstantivfarbstoffen; und Mischungen davon.

3. Flüssige Zusammensetzung nach einem der vorstehenden Ansprüche, wobei mindestens 90 %, vorzugsweise 95 % der Teilchen, bezogen auf die Anzahl, eine Länge von weniger als 6 Mikrometern besitzen.

4. Flüssige Zusammensetzung nach einem der vorstehenden Ansprüche, wobei das nichtpolymere, kristalline, hydroxylhaltige Strukturierungsmittel gehärtetes Rizinusöl ist.

5. Einheitsdosisartikel, umfassend eine flüssige Waschmittelzusammensetzung nach einem der Ansprüche 1 bis 2, wobei die flüssige Waschmittelzusammensetzung weniger als 20 Gew.-% Wasser umfasst und in einer wasserlöslichen Folie eingekapselt ist.

## Revendications

1. Composition liquide, comprenant un prémélange structurant aqueux,
dans laquelle ledit prémélange structurant aqueux comprend de l'eau et des particules, lesdites particules comprenant un agent structurant non polymère, cristallin, contenant un hydroxyle, dans laquelle au moins 80 % en nombre des particules ont une longueur inférieure à 6 micromètres ;
où la composition liquide est une composition détergente liquide, comprenant au moins un agent tensioactif, présent à un taux allant de 1 à 70 % en poids de la composition liquide ; et
où la composition liquide comprend de 0,01 % en poids à 2 % en poids de l'agent structurant non polymère, cristallin, contenant un hydroxyle, introduit par l'intermédiaire du prémélange structurant aqueux.

2. Composition liquide selon la revendication 1, où la composition détergente liquide comprend en outre des ingrédients détergents choisis dans le groupe constitué de : agents tensioactifs supplémentaires choisis parmi un agent tensioactif amphotère, zwittérionique, cationique, et des mélanges de ceux-ci ; des enzymes ; des agents stabilisant les enzymes ; des polymères de nettoyage de la graisse alcoxylés amphiphiles ; des polymères de nettoyage de salissures d'argile ; des polymères antisalissures ; des polymères de suspension des salissures ; des systèmes de blanchiment ; des azurants optiques ; des teintures teintantes ; des matières particulaires ; des parfums et d'autres agents de lutte contre les odeurs, y compris des systèmes de libération de parfum ; des hydrotropes ; des suppresseurs de mousse ; des parfums pour le soin des tissus ; des agents d'ajustement du pH ; des agents inhibant la décoloration ; des conservateurs ; des teintures non substantives sur les tissus ; et des mélanges de ceux-ci.

3. Composition liquide selon l'une quelconque des revendications précédentes, dans laquelle au moins 90 %, de préférence 95 % en nombre des particules ont une longueur inférieure à 6 micromètres.

4. Composition liquide selon l'une quelconque des revendications précédentes, dans laquelle l'agent structurant non polymère, cristallin, contenant un hydroxyle est l'huile de ricin hydrogénée.

5. Article en dose unitaire, comprenant une composition détergente liquide selon l'une quelconque des revendications 1 à 2, dans lequel la composition détergente liquide comprend moins de 20 % en poids d'eau, et est encapsulée dans un film hydrosoluble.
